# EUROPEAN PATENT SPECIFICATION

(11) **EP 0 520 023 B1**
(45) Date of publication and mention of the grant of the patent: **24.05.1995**
(21) Application number: 91906840.3
(22) Date of filing: 06.03.1991
(51) Int. Cl.: D02G 3/04, D01F 6/04

(54) **SPINNING OF HIGH MOLECULAR WEIGHT POLYETHYLENE FIBER AND THE RESULTING SPUN FIBER**
VERSPINNEN VON HOCHMOLEKULARER POLYÄTHYLENFASER UND DARAUS RESULTIERENDE FASER
FILAGE D'UNE FIBRE POLYETHYLENE DE POIDS MOLECULAIRE ELEVE ET FILE AINSI OBTENU

(30) Priority: 14.03.1990 US 493178
(43) Date of publication of application: 30.12.1992
(73) Proprietor: AlliedSignal Inc., Morristown, New Jersey 07962-2245 (US)
(72) Inventor: KIRKLAND, Kevin, Mark, Richmond, VA 23235 (US); WEBER, Charles, Paul, Jr., Monroe, NC 28110 (US)
(74) Representative: Lawrence, Peter Robin Broughton
(86) International application number: US9101561
(87) International publication number: WO9114029

(56) References cited:
- EP-A- 310 202
- GB-A-21 525 43
- US-A- 4 457 985

## Description

### 1. Field of the Invention

The present invention relates to the spinning of staple fibers into yarn and to the resulting spun yarn. More particularly, it relates to the spinning of high molecular weight polyethylene staple fiber and to modifications to conventional spinning technology necessary to spin the high molecular weight polyethylene fiber.

### 2. The Prior Art

The spinning of staple (discontinuous lengths) fibers has been practiced for centuries. Natural fibers are of discontinuous lengths and require spinning to form a continuous yarn. Synthetic continuous filament fibers are converted into staple fiber and spun for a variety of reasons. One such reason is to improve the hand or appearance of the yarn. Another reason is to make a good yarn less expensively since the spinning process permits the use of some fiber which would have been wasted.

With the advent of the high molecular weight polyethylene continuous filament fibers which are produced by solution spinning, such as SPECTRA high strength polyethylene fiber, it was only a matter of time before an attempt was made to cut the continuous filament fiber into staple and spin the staple fiber a fiber into yarn. When the attempt was made, it was not possible to card the fiber since the fiber batt was so slippery that it could not be moved by the conventional feed roll to the card. Furthermore, when an attempt was made to overcome the slipperiness problem by crimping the fiber, it was found that the fiber would not hold crimp. Another reason to attempt crimping was that the high strength polyethylene fibers would not spring back from being compressed during normal spinning processing, which is contrary to experience with other fibers. Until this invention that problem was not solved. The present invention was developed to overcome these problems.

There have been disclosures of polyolefin fibers blended with other fibers, but none of these disclosures focuses on high molecular weight polyethylene staple fiber. For example, EP-A-0 310 202 describes combining polyolefin filament or yarns with filaments or yarns having high wetting and adhesive power. The filaments or yarns are combined by core spinning or twisting and there is no mention that a spun yarn could be formed from staple fibers of this combination. GB-A-2 152 543 discloses a high bulk olefin blended yarn which includes olefin fiber and a naturally occurring fiber such as cotton or wool. There is no mention of solution or gel spun high molecular weight polyethylene fiber.

### BRIEF DESCRIPTION OF THE INVENTION

This invention is a spun yarn, comprising discontinuous lengths of a high molecular weight polyethylene fiber and a sufficient amount of discontinuous lengths of any other fiber to permit spinning a blend of the fiber lengths.

The molecular weight of the polyethylene is greater than 300,000, and more preferred is the molecular weight of greater than 500,000.

The preferred other fiber has memory. By memory is meant ability to return to original shape after distortion. For example a straightened, formerly crimped fiber that will return to its original crimped state.

The preferred other fiber has a denier per filament of no greater than 20 (180 tex), more preferably the other fiber has a denier per filament of no greater than 3 (27 tex).

The preferred discontinuous lengths of the polyethylene fiber and the other fiber are no longer than 14 inches (35.6 cm), more preferably the discontinuous lengths of the polyethylene fiber and the other fiber have a length ranging from 0.75 to 14 inches (1.9 to 35.6 cm).

The polyethylene fiber forms 5 to 95% by weight of the spun fiber, more preferably, the polyethylene fiber forms 5 to 60% by weight of the spun fiber.

Preferably, the polyethylene fiber has an ultimate elongation of less than 8% at room temperature, more preferably 2 to 4.5%. Preferably the polyethylene fiber has a denier per filament of no greater than 20 (180 tex), more preferably 1 to 15 (9 to 135 tex), and most preferably, 1 to 10 (9 to 90 tex). Even more preferably the polyethylene fiber has a denier per filament of 1 to 3 (9 to 27 tex).

The preferred other fiber is selected from the group consisting of polyester fiber, polyamide fiber, cotton fiber, wool fiber, rayon fiber, polypropylene fiber, aramid fiber, lower molecular weight polyethylene fibers, carbon fiber, and mixtures thereof.

It is preferred that the other fiber, forming 5 to 95% by weight of the spun fiber, is characterized by having memory, a denier per filament of no more than 20 (180 tex), and discontinuous lengths of no more than 14 inches (35.6 cm).

It is preferred that polyethylene fiber forming 5 to 95% by weight of the spun fiber, is characterized by an elongation of no more than 8% at room temperature, a denier per filament of no more than 20 (180 tex), and discontinuous lengths of no more than 14 inches (35.6 cm).

It is more preferred that the other fiber is an aramid fiber which forms no more than 50% by weight of the spun fiber.

The preferred aramid other fiber is poly(p-phenylene terephthalamide).

Use of lower price other fiber can create lower cost yarn blends.

This invention is also an article made from the spun yarn of the spun fiber described above, preferably the article made from the spun fiber of 50% aramid.

This invention is also a method of spinning discontinuous lengths of a high molecular weight polyethylene fiber, comprising blending a sufficient amount of discontinuous lengths of any other fiber to permit spinning of a blend of the fiber lengths.

The preferred and more preferred molecular weights of the polyethylene are given above, along with the preferred, more preferred percent by weight blends, fiber weights, other fiber types, elongations, etc.

This invention is also an apparatus for moving a fiber batt of at least 50 weight percent high molecular weight polyethylene fiber, comprising rotating means, said rotating means having a surface which rotates into contact with said fiber batt, and a cord aligned with a trumpet to form the fiber batt into a sliver, said surface being modified across at least a portion thereof to increase the friction between the surface and the fiber batt so that the batt moves when contacted by the rotating surface. The trumpet has an exit for the sliver sufficiently enlarged to limit compression of the sliver to the extent that it can be piddled.

It is preferred that the surface be modified by having an adhesive across said portion, a double-backed tape across said portion, or fabric capable of increasing friction or engaging the fiber (such as a Velcro tape or Emory cloth) attached to said portion.

The surface also can be modified by roughening to a surface of roughness of similar to 800 grit sandpaper or more coarse.

### BRIEF DESCRIPTION OF THE DRAWINGS

In the accompanying drawings,
FIGURE 1 is a schematic overview of the prior art cotton carding process for sliver production;
FIGURE 2 is a detail of the card from FIGURE 1;
FIGURE 3 is a detail of the feed to the card, with emphasis on feed to the lickerin;
FIGURE 4 is a detail of the modified feed roll 23;
FIGURE 5 has various views of trumpet 21.
FIGURE 5A is an isometric view of a prior art trumpet shown in section in FIGURE 5B; and FIGURE 5C is a section of a modified trumpet, showing the enlarged exit opening. FIGURE 5D is an end view.

### DETAILED DESCRIPTION OF THE INVENTION

In the accompanying drawings, like numbers refer to like apparatus. The process which is depicted and which was used in the examples which follow was the cotton system of spinning yarn. For more detail on this system, reference may be had to Textile Processing Vol. I by John H. Marvin, (1973) - South Carolina State Dept. of Education Office of Vocational Education; and Textiles: Fiber to Fabric by M.D. Potter and B.P. Corbman (1975) - McGraw-Hill Inc., see Chpt. 3 pp 35 to 71.

With reference to FIGURE 1, discontinuous fiber lengths, here staple, are placed by an operator into the backs of a plurality of hoppers 11. Inside each hopper 11, the individual mass of fibers is broken into smaller tufts by spiked conveying aprons (not shown) which then feed the tufts onto conveyor belt 12 to mix with tufts of fibers from other hoppers 11. Conveyor belt 12 then feeds the mixture of fibers into a blending unit 13 where they are further broken into smaller elements and further mixed. From unit 13 the fibers are transported through pipe 15 via Whitin Axi-Flo Unit 14 which is a pneumatic system, to pneumatic distributor 16. Distributor 16 further opens and fluffs the fibrous mass and then meters the fiber into the CMC Evenfeed Unit 17 which begins to form the fiber batt 35 from fiber 24 (referred to as a fiber lap in the art). With reference to Fig. 1, Fig. 2, Fig. 3 and FIGURE 5, fiber batt 35 is fed via feed plate 37 in association with feed roll 23 to lickerin 22 which has a plurality of wires 50 (card cloth) which rotate against batt 35 to pull and align discrete fibers from batt 35 and transfer them to the card cloth 50 covering the card cylinder 33 where they are further oriented and worked (brushed/combed) by the carding plates or flats 25. Doffer 30 is also covered with a card cloth, removes the accumulating sheet of oriented fibers from card 18 and carries the sheet of fibers to a removal point where it can be removed by a comb 28. The sheet of fibers is then fed through a trumpet 21 which forces the sheet to neck down for passage through a circular aperture 54. From aperture 54, the sliver 20 (necked down fiber sheet) is piddled into a take-up can 19 where it is loosely coiled.

The modification to feed roll 23 is shown in Fig. 4; double-sided adhesive tape 52 was spiralled around roll 23, as shown. Without use of an adhesive such as the tape, or another surface modification the feed roll does not function properly when high strength, high molecular weight polyethylene staple fiber is being processed, especially when blends over about 50% high molecular weight polyethylene are being processed. Without modification, the batt of fibers just slips and backs up, forms clumps and therefore the machine must be stopped because the fiber can not be carded.

Figs. 2,3,4 and 5 provide more detail regarding the prior art process showing feed roll 23 and surrounding members in greater detail.

Fig. 2 shows feed plate 37, card cylinder 33 screen 38, having wire 50 protruding, lickerin screen 40, backplate 34, spiral brush 31 for flats 25, front plate 29. Calender rolls 27 convey the sliver 20 from trumpet 21 to sliver can 19 on holder 26. Clearer 43, clears feed roll 23. Lap guide 45 guides the lap to feed roll 23. Mote knives 48 cut away motes which may accumulate from the lap.

Fig. 5 shows trumpet 21 in various aspects. Figure 5A is an isometric view and Fig. 5B is a cross section showing outlet opening 54 while 5D shows end view of trumpet 21 having outer perimeter 55 and outlet 54. Fig. 5C show the enlarged outlet opening 57, necessary for production of the spun fiber of this invention. For further reference to the general discussion which follows, refer to Textile Processing Vol.I, supra.

As previously indicated, when an attempt was made to spin staple high molecular weight polyethylene fiber alone with the system depicted in the drawing figures, feed roll 23 could not move batt 35 forward to the lickerin. Two modifications were made. The fiber was blended with other fiber, to be discussed in more detail below, and the feed roll 23 was modified as shown in FIGURE 4 with a spiral of double-backed masking tape on its surface that rotates into contact with batt 35 to permit it to move batt 35 forward. Anything that can be put on the feed roll 23 to enchance the frictional characteristics between its surface and batt 35 is acceptable, and it may be coextensive with the roll surface or distributed over a portion thereof as long as the batt 18 can be moved by it. For example, Velcro - type tape, Emery cloth, a roughened surface, adhesive, double-backed tape or the like can be used.

Another problem was encountered at trumpet 21. Due to the inability of the fiber to hold crimp, it does not spring back after deformation. After the neck down of trumpet 21 aperture 28, the sliver 20 is like a rod and difficult to piddle. Therefore, trumpet 21 was bored out sufficiently to increase the size of the sliver 20 and to reduce or limit the compression of the sliver to the extent that it could be piddled (see FIGURE 5C).

Cans of the attenuated sliver are collected and transferred to a draw frame, in the accompanying examples a Saco Lowell four over five draw frame, where several individual slivers are blended and further attenuated/drawn.

The cans of attenuated, blended sliver are then transferred to a roving frame for further attenuation and a very low level of twist is inserted. The sliver is now ready for spinning and is taken-up on a bobbin which is the feeder package for the spinning frame.

The bobbins are hung on a spinning frame, preferably a ring spinning frame, where the slivers are again individually attenuated and spun into yarn by twisting. The spun yarn is then taken up for packaging or further processing.

US-A-4,457,985, generally discusses high molecular weight polyethylene. In the case of polyethylene, suitable fibers are those of molecular weight of at least 300,000, more preferably at least 500,000, most preferably in excess of one million. Such extended chain polyethylene (ECPE) fibers may be grown in solution as described in US-A-4,137,394 or US-A-4,356,138, or may be a filament spun from a solution to form a gel structure, as described in DE-A-3,004,699 and GB-A-2,051,667, and especially described in US-A-4,551,296. As used herein, the term polyethylene shall mean a predominantly linear polyethylene material that may contain minor amounts of chain branching or comonomers not exceeding 5 modifying units per 100 main chain carbon atoms, and that may also contain admixed therewith not more than 50 weight percent of one or more polymeric additives such as alkene-1-polymers, in particular low density polyethylene, polypropylene or polybutylene, copolymers containing mono-olefins as primary monomers, oxidized polyolefins, graft polyolefin copolymers and polyoxymethylenes, or low molecular weight additives such as lubricants, colorants, fillers and the like which are commonly incorporated by reference. Depending upon the formation technique, the draw ratio and temperatures, and other conditions, a variety of properties can be imparted to these filaments. The tenacity of the filaments should be at least 8 g/d (7.1 dN/tex), preferably in the range of from 8 to 45 g/d (7.1 to 39.7 dN/tex), most preferably in the range of 25 to 35 g/d/ (22.1 to 30.9 dN/tex). Similarly, the tensile modulus of the filaments, as measured by an Instron tensile testing machine, is at least 160 g/d (141.3 dN/tex), preferably in the range of 150 to 3300 g/d (132.5 to 2913.9 dN/tex), most preferably in the range of 1,200 to 2,500 g/d (1059.6 to 2207.5 dN/tex). These highest values for tensile modulus and tenacity are generally obtainable only by employing solution grown or solution spun, gel filament processes.

The polyethylene fiber should preferably have an ultimate elongation by Instron tensile test of no greater than 8%, preferably in range of 2 to 4.5%, at room temperature, i.e., about 25° C. The denier per filament is preferably no greater than 20 (180 tex), more preferably 1 to 15 (9 to 135 tex), most preferably 1 to 10 (9 to 90 tex), even more preferably 1 to 3 (9 to 27 tex). The smaller denier per filament fibers are desirable to use in spinning blends for apparel applications. The larger denier per filament fibers are better to use in spinning blends for cordage, ropes, or heavy fabric applications.

The amount of polyethylene fiber in the blend ranges from about 5 to 95% by weight, preferably 20 to 80 % by weight as the primary fiber and 5 to 40% by weight as the support fiber.

The carrier fiber may be any other fiber. i.e., anything except the high molecular weight polyethylene fiber just described. Exemplary fibers may be found listed in allowed U.S. Patent Application S.N. 62,998 filed July 13, 1987, now US-A-4 916 000. A partial listing would include the aramids, cottons, carbon, polyester, polyamides, wool, rayon, polypropylene, lower molecular weight polyethylenes, etc.

The carrier fiber preferably should have the following characteristics: it should preferably be a fiber which has memory or is permanently crimped; it should preferably have a denier per filament of no greater than 20 (180 tex), more preferably 0.5 to 3 (4.5 to 27 tex) for apparel applications and preferably 3 to 20 (27 to 180 tex) for ropes, cordage, and heavy fabric applications.

The minimum amount of carrier fiber needed is 5% by weight of the spun fiber, and up to 95% by weight is acceptable. The preferred amount will range from about 20 to 50% by weight. The amount will be a function of the denier of the polyethylene fiber, e.g. one would need about 30% by weight carrier fiber to spin a 20 denier (180 tex) per filament polyethylene fiber, and would need less to spin a lower denier per filament polyethylene fiber.

Both the carrier fiber and the polyethylene fiber are formed from discontinuous lengths of no greater than about 14 inches (35.6 cm), preferably no longer than 2.25 inches (5.7 cm) in the cotton system, more preferably 0.75 to 2 inches (1.9 to 5.1 cm).

The particular blends of carrier fibers will depend on desired properties of the spun fiber. It is contemplated that a blend of polyester and/or cotton with the polyethylene will enhance hand; polypropylene can be blended for pigmentation; aramids, specifically Kevlar and Nomex can be includes for flame resistance; polybenzimidazoles (PBI), avilable commercially from Hoechst-Celanese, can be included for flame resistance and enchanced comfort due to higher moisture regain; carbon for use in fiber for composites requiring strength and toughness. Activated carbon fiber could be used for chemical absorption protection.

### EXAMPLES

### EXAMPLE 1 (including comparative)

Using the apparatus of Fig. 1, a two-inch (5.1 cm) SPECTRA 900 fiber available from Allied-Signal Inc. is run on the apparatus, unsuccessfully. The fiber slips on the feed rolls, clumps up in the feed mechanism and the machine must be stopped. A second trial was attempted with a fiber blend of 70% of the SPECTRA 10 dpf (90 tex) fiber above and 30% 1.2 denier (10.8 tex) per filament (dpf) Kodel polyester 1.5 inch (3.8 cm) staple. The mixture of 70% Spectra 10 dpf (90 tex) two inch (5.1 cm) staple and 30% 1.2 dpf (10.8 tex) Kodel 1.5 inch (3.8 cm) polyester staple was prepared and loaded into the card feeder. Difficulty in carding the fiber mixture was encountered after about 30 minutes because the polyester fiber rolled on itself and formed small balls of fiber. The screen inside the Even Feed unit could not move the bat of Spectra fiber and the balls of polyester fiber to the card main cylinder. The fiber bat was probably too slippery to be moved by the feeder mechanism. The trial was terminated and the card feeder was cleaned.

The second trial was conducted using a blend by weight of 60% Spectra 900 10 dpf (90 tex) 2.0 inch (5.1 cm) staple fiber and 40% Kevlar 1.5 dpf (13.5 tex) 1.5 inch (3.8 cm) staple fiber. A length of double-backed adhesive tape was spirally wrapped around feed roll 23 as in Fig. 4. The difference in the two fibers dpf caused some problems with how well the mixture blended and carded. The problems were not serious. However, to optimize the process it may be desirable to have fibers which have similar dpf.

A total of 50 pounds (22.7 kg) of Spectra/Kevlar fiber blend was made. To control static electricity Stay Guard antistatic spray was purchased from a local grocery store. The anti static spray was added to the fiber in the opener as the fiber was being opened and blended. There were no static electricity problems.

The main problem encountered during carding was the loading of the card main cylinder by the Spectra fiber. This problem may be solved by using a fiber with a smaller dpf or development of a special fiber finish. There was also a large amount of Spectra fiber removed by the card flats. The card flats rotate against the main cylinder to help clean it. This problem may disappear if the cylinder loading problem can be solved.

The carded sliver was divided into six ends which were fed into a Saco Lowell 4 over 5 draw frame. The draw frame was running black coated rubber rolls. The black rolls seemed to minimize the tendency of the sliver to wrap. The draw frame further blended the carded sliver and reduced the sliver weight by about 50%.

The roving was produced on a Saco Lowell roving frame. No problems were encountered during the roving formation.

The roving was converted to spun yarn on a ring spinning frame. The speeds and conditions were varied to produce a yarn which had a specific cotton count. The first yarn count attempted was a 20's.

The spinning of the 20's yarn was very difficult because the yarn kept breaking. A calculation showed that because of the fiber diameters, the formation of a 20's count yarn was on the edge of being a physical impossibility. (Theoretically, at least 88 fibers are required in the cross section of a spun yarn. Because of the dpf of the Spectra fiber, it is impossible to have enough fiber in the spun yarn cross section and the yarn still be small enough to be a 20's.)

The two spun yarns produced were a 10's and a 5's cotton count. Both of these yarns spun easily. Some optimization will be necessary to achieve the best balance of physical properties in the finished yarn.

### EXAMPLE 2

Example 1 was repeated loading the following fibers:
70% of 3 dpf (27 tex) SPECTRA * 2" (5.1 cm) staple
30% of 1.2 dpf (10.8 tex) Kodel polyester 1.5" (3.8 cm) staple Four spun yarns were successfuly produced:
10 cotton count single, 10 cotton count two-ply,
20 cotton count single, 20 cotton count two-ply.
*The SPECTRA fiber had a lower intrinsic viscosity of between 6 and 8, estimated molecular weight about 700,000.

### EXAMPLE 3 (Comparative)

An attempt to spin 100% SPECTRA fiber on the unmodified apparatus of Example 1 was unsuccessful, as was another attempt on a worsted spinning system.

### SPECTRA / ARAMID BLEND SPUN YARN GLOVE

The article made from the blond of Spectra and Kevlar fiber from Example #1 exhibited good flame resistance and insulating properties. When the fabric (in this cane a knitted glove) was exposed to a flame from a cigarette lighter the exposed polyethylene fibers on the fabric surface melted back into the fabric even with the aramid fiber surface. The fabric did not ignite or burn which in surprising because Spectra fiber is a polyolefin which will burn if it becomes hot enough. The inside of the glove remained cool. The Spectra fibers did not seem to melt on the side of the fabric opposite the flame. When an attempt to intentionally ignite the fabric made from the blend of Spectra and aramid fibers was made the fabric exhibited a self extinguishing behavior and did not readily support combustion. (Surprising because olefin fibers are known to burn).

The Spectra fiber should improve the abrasion resistance of the aramid fiber (in the case of the glove) and allow the item to have a longer service life. The fabric made from the blend of fibers had a good hand and the frictional characteristics of the fabric surface were improved over an all Spectra fabric because the aramid fiber reduced the slickness of the surface. This improved frictional property would be desirable in a glove because of the necessity of keeping a good grip on objects being handled.

## Claims

1. A spun yarn comprising discontinuous lengths of at least two different types of fibers, characterized in that one fiber type is a solution or gel spun polyethylene fiber having a molecular weight of greater than 300,000 and the second fiber type or types is any other fiber which is present in an amount from 5 to 95% by weight, based on spun fiber, and sufficient to permit spinning a blend of the different fiber types.

2. The yarn of claim 1 wherein the other fiber has memory.

3. The yarn of claim 1 wherein the other fiber has a denier per filament of no greater than 20 (180 tex).

4. The yarn of claim 1 wherein the other fiber is selected from the group consisting of polyester fiber, polyamide fiber, cotton fiber, wool fiber, rayon fiber, polypropylene fiber, aramid fiber, lower molecular weight polyethylene fibers, carbon fiber, and mixtures thereof.

5. The yarn of claim 2 wherein the other fiber is an aramid fiber which forms no more than 50% by weight of the spun fiber.

6. The yarn of claim 2 wherein the other fiber is poly (p-phenylene terephthalamide).

7. An article made from a spun yarn comprising discontinuous lengths of at least two different types of fibers, characterized in that one fiber type is a solution or gel spun polyethylene fiber having a molecular weight of greater than 300,000 and the second fiber type or types is any other fiber which is present in an amount from 5 to 95% by weight, based on spun fiber, and sufficient to permit spinning a blend of the different fiber types.

8. A method of spinning discontinuous lengths of at least two different types of fibers, characterized by (a) blending 5 to 95% by weight of discontinuous lengths of a solution or gel spun polyethylene fiber having a molecular weight of greater than 300,000 with a sufficient amount of discontinuous lengths of any other fiber to permit spinning of the blend, and (b) spinning the resultant blend to form a yarn.

9. The method of claim 8 wherein the other fiber is selected from the group consisting of polyester fiber, polyamide fiber, cotton fiber, wool fiber, rayon fiber, polypropylene fiber, aramid fiber, lower molecular weight polyethylene fibers, carbon fiber, and mixtures thereof.

10. An apparatus for transporting a fiber batt (35) of at least 50 weight percent high molecular weight polyethylene fiber which includes a rotating means (23) having a surface which rotates into contact with the fiber batt (35) and a card (18) aligned with a trumpet (21) to form the fiber batt (35) into a sliver (20), wherein at least a portion of the surface is characterized by being modified to increase the friction between the surface and the fiber batt (35) and the trumpet (21) is characterized by having an exit (57) for the sliver (20) sufficiently enlarged to limit compression of the sliver to the extent that it can be piddled.

## Patentansprüche

1. Gesponnenes Garn mit diskontinuierlichen Längen wenigstens zweier unterschiedlicher Arten von Fasern, dadurch gekennzeichnet, daß die eine Faser ein lösungs- oder gelgesponnene Poläthylenfaser mit hohem Molekulargewicht von mehr als 300 000 ist und die zweite Faserart oder -arten jede andere Faser ist, welche in einer ausreichenden Menge vorhanden ist, um das Spinnen einer Mischung der unterschiedlichen Faserarten zu erlauben.

2. Garn nach Anspruch 1, bei dem die andere Faser ein Gedächtnis aufweist.

3. Garn nach Anspruch 1, bei dem die andere Faser eine nicht größere Denierzahl pro Filament aufweist als etwa 20.

4. Garn nach Anspruch 1, bei dem die andere Faser aus der aus Polyesterfasern, Polyamidfasern, Baumwollfasern, Wollfasern, Rayonfasern, Polypropylenfasern, Aramidfasern, Polyäthylenfasern niedrigeren Molekulargewichtes, Kohlenstoffasern und Gemischen davon bestehenden Gruppe ausgewählt ist.

5. Garn nach Anspruch 2, bei dem die andere Faser eine Aramidfaser ist, die nicht mehr als etwa 50 Gewichts-% der gesponnenen Faser ausmacht.

6. Garn nach Anspruch 2, bei dem die andere Faser Poly(p-Phenylen-Terephthalamid) ist.

7. Gegenstand, der aus einem gesponnenen Garn mit diskontinuierlichen Längen wenigstens zweier unterschiedlicher Arten von Fasern hergestellt ist, dadurch gekennzeichnet, daß eine Faserart eine lösungs- oder gelgesponnene Poläthylenfaser mit hohem Molekulargewicht von mehr als 300 000 ist und die zweite Faserart oder -arten jede andere Faser ist, welche in einer ausreichenden Menge vorhanden ist, um das Spinnen einer Mischung der unterschiedlichen Faserarten zu erlauben.

8. Verfahren zum Spinnen diskontinuierlicher Längen wenigstens zweier unterschiedlicher Arten von Fasern, gekennzeichnet durch (a) Mischen von 5 bis 95 Gewichts-% von diskontinuierlicher Längen einer lösungs- oder gelgesponnenen Polyäthylenfaser mit einem höheren Molekulargewicht als 300 000 mit einer ausreichenden Menge an diskontinuierlichen Längen einer anderen Faser, um das Spinnen der Mischung zu erlauben, und (b) Verspinnen der sich ergebenden Mischung zur Bildung eines Garnes.

9. Verfahren nach Anspruch 8, bei dem die andere Faser aus der aus Polyesterfasern, Polyamidfasern, Baumwollfasern, Wollfasern, Rayonfasern, Polypropylenfasern, Aramidfasern, Polyäthylenfasern niedrigeren Molekulargewichtes, Kohlenstoffasern und Gemischen davon bestehenden Gruppe ausgewählt ist.

10. Vorrichtung zum Transportieren einer Faserflocke (35) von wenigstens 50 Gewichtsprozent einer Polyäthylenfaser hohen Molekulargewichtes, welche eine Dreheinrichtung (23) mit einer Oberfläche aufweist, die sich in Berührung mit der Faserflocke (35) und eine Karde (18) welche zur Bildung der Flocke zu einer Lunte in einer Linie mit einem Einfülltrichter (21) liegt, wobei wenigstens ein Teil der Oberfläche so abgeändert ist, daß die Reibung zwischen der Oberfläche und der Faserflocke (35) erhöht wird, und der Einfülltrichter (21) dadurch gekennzeichnet ist, daß er einen vergrößerten Ausgang (57) für die Lunte (20) aufweist.

## Revendications

1. Filé comprenant des tronçons discontinus d'au moins deux types de fibres différents, caractérisé en ce qu'un type de fibre est une fibre de polyéthylène filée en solution ou en gel ayant une masse moléculaire supérieure à 300 000 et le second type ou les types de fibre sont tout autre fibre qui est présente dans une quantité suffisante pour permettre le filage d'un mélange des types de fibres différents.

2. Filé selon la revendication 1, dans lequel l'autre fibre a de la mémoire.

3. Filé selon la revendication 1, dans lequel l'autre fibre a un denier par filament non supérieur à environ 20.

4. Filé selon la revendication 1, dans lequel l'autre fibre est choisi dans le groupe constitué d'une fibre de polyester, d'une fibre de polyamide, d'une fibre de coton, d'une fibre de laine, d'une fibre de rayonne, d'une fibre de polypropylène, d'une fibre d'aramide, de fibres de polyéthylène à faible masse moléculaire, d'une fibre de carbone, et de leurs mélanges.

5. Filé selon la revendication 2, dans lequel l'autre fibre est une fibre d'aramide qui ne constitue pas plus d'environ 50 % en poids de la fibre filée.

6. Filé selon la revendication 2, dans lequel l'autre fibre est le poly(téréphtalamide de p-phénylène).

7. Article réalisé avec un filé comprenant des tronçons discontinus d'au moins deux types différents de fibres, caractérisé en ce qu'un type de fibre est une fibre de polyéthylène filée en solution ou en gel ayant une masse moléculaire supérieure à 300 000 et le second type ou les seconds types de fibres sont tout autre fibre qui est présente dans une quantité suffisante pour permettre le filage d'un mélange des types de fibres différents.

8. Procédé pour filer des tronçons discontinus d'au moins deux types de fibres différents, caractérisé par (a) le mélange de 5 à 95 % en poids de tronçons discontinus d'une fibre de polyéthylène filée en solution ou en gel ayant une masse moléculaire supérieure à 300 000 avec une quantité suffisante de tronçons discontinus de tout autre fibre afin de permettre le filage du mélange, et (b) le filage du mélange obtenu afin de former un filé.

9. Procédé selon la revendication 8, dans lequel l'autre fibre est choisie dans le groupe constitué d'une fibre de polyester, d'une fibre de polyamide, d'une fibre de coton, d'une fibre de laine, d'une fibre de rayonne, d'une fibre de polypropylène, d'une fibre d'aramide, de fibres de polyéthylène à faible masse moléculaire, d'une fibre de carbone, et de leurs mélanges.

10. Dispositif pour transporter une galette de fibres (35) d'au moins 50 % en poids d'une fibre de polyéthylène de masse moléculaire élevée qui comprend un moyen tournant (23) ayant une surface qui tourne en contact avec la galette de fibres (35) et une carde (18) en alignement avec un entonnoir de filature (21) pour transformer la galette de fibres (35) en une mèche (20), dans lequel au moins une partie de la surface est caractérisée en ce qu'elle est modifiée de manière à augmenter la friction entre la surface et la galette de fibres (35) et l'entonnoir de filature (21) est caractérisé en ce qu'il comporte une sortie agrandie (57) pour la mèche (20).
